

# United States Patent Office

3,728,164

Patented Apr. 17, 1973

1

3,728,164

## METHOD FOR FORMING A CHEMICAL COATING ON ALUMINUM OR ALUMINUM ALLOY

Takashi Abe, Koji Aizawa, and Masanobu Oguri, Osaka, Japan, assignors to Showa Aluminium Kabushiki Kaisha, Osaka, Japan

No Drawing. Filed Sept. 23, 1970, Ser. No. 74,837  
Claims priority, application Japan, Oct. 13, 1969,

44/82,122

Int. Cl. C23f 7/06

U.S. Cl. 148—6.27

1 Claim 10

### ABSTRACT OF THE DISCLOSURE

A method for forming a chemical coating on aluminum or aluminum alloy in which the aluminum or aluminum alloy is immersed in an aqueous solution containing monoethylamine or diethylamine. The aqueous solution can be heated either before or after the addition of monoethylamine or diethylamine. After immersing, the metal may be subjected to pressurized steam.

### BACKGROUND AND SUMMARY

The present invention relates to a method for forming a chemical coating on aluminum or aluminum alloy (hereinafter referred to as "aluminum"). The coating so formed contains boehmite, i.e., hard, crystalline water-insoluble  $\text{AlOOH}$ .

Since aluminum has come to be employed for versatile uses in recent years, there arises a need to subject aluminum to some surface treatment to enhance durability. Accordingly, various methods of surface treatment such as anodic oxidation processes for providing electrochemical coating, or MBV process, Alodine process, etc. for forming chemical coating are used depending upon the purposes. However, anodic oxidation process has drawbacks in that it requires complex electrical equipments and in that distribution of electricity is not necessarily effected uniformly depending upon the shape of articles with the result that some portions are left uncoated even after treatment. On the other hand, MBV and Alodine processes, though generally used, are not satisfactory because the coating is poor in corrosion resistance. Also known in recent years is the boehmite process in which aluminum is immersed in a boiling aqueous solution containing triethanolamine, monoethanolamine or the like to form a chemical coating, but the coating thus formed is generally thin and therefore it is desired to improve its corrosion resistance.

In view of the above, the present invention contemplates providing a uniform and corrosion-resistant coating without using a complex apparatus, the invention being characterized in that aluminum is treated by being immersed in a boiling aqueous solution containing at least one member selected from the class of monoethylamine and diethylamine.

### DETAILED DESCRIPTION OF THE INVENTION

In more detailed description, the present invention is accomplished by immersing aluminum for several tens of minutes in a solution in boiling or resembling state prepared by adding monoethylamine, diethylamine or both amines to pure water or distilled water. The water may be heated to boiling before or after the addition of the amine.

The amount of the amine to be added at this time may preferably be about 0.5 cc./liter, to 30 cc./liter. If the amount is smaller than 0.5 cc./liter, satisfactory corrosion resistance will not be obtained, while the addition of more than 30 cc./liter results in hardly any noticeable effect but rather expedites deterioration of the treating solution.

2

Further prior to the treatment of the present invention, an ordinary pretreatment such as washing or removal of oily substances on the surface of aluminum is performed, while the present treatment is followed by an aftertreatment employing pressurized steam or the like.

Examples of the present invention will be given below.

### EXAMPLE 1

In order to remove oil and fat and oxidized film from the surface of aluminum for cleaning, aluminum was immersed for 2 minutes in a 5% solution of caustic soda heated to 80°C. and then washed with water. The aluminum was thereafter immersed for 30 seconds in a 30% nitric acid solution for neutralization and washed with water. After this pretreatment, 1100 aluminum plates (1 mm. x 56 mm. x 100 mm.) obtained were subjected to a treatment in accordance with the present invention by immersing them for 30 minutes and 60 minutes respectively in a boiling aqueous solution which was prepared by adding 3 cc./liter of monoethylamine to pure water. Aftertreatment was conducted for 20 minutes in a pressurized steam of 4 kg./cm.<sup>2</sup>. The number designation herein used refers to the Aluminum Association Standard Number for wrought aluminum alloy.

The same treatments were carried out in the same manner as above except that diethylamine, and both amines of monoethylamine and diethylamine were used in place of monoethylamine. The ratio of monoethylamine and diethylamine was about 1:1.

The aluminum plates chemically treated in the above-mentioned manner were tested to measure the weight of the coating and resistance to alkali and to acid. The results are stated below.

As reference examples the results obtained by using monoethanolamine, triethanolamine, triethylamine and triallylamine are also given. The treating conditions in these cases were exactly the same as those in the case of monoethylamine.

#### (1) Measurement of weight of coating

The weight of the coating was measured to observe the state of the coating formed.

| Additives                            | Treating time (min.) | Weight of coating (mg./dm. <sup>2</sup> ) |
|--------------------------------------|----------------------|-------------------------------------------|
| Present invention:                   |                      |                                           |
| Monoethylamine.....                  | 30                   | 57.0                                      |
|                                      | 60                   | 58.4                                      |
| Diethylamine.....                    | 30                   | 33.4                                      |
|                                      | 60                   | 35.2                                      |
| Monoethylamine and diethylamine..... | 30                   | 50.4                                      |
|                                      | 60                   | 52.0                                      |
| Reference examples:                  |                      |                                           |
| Monoethanolamine.....                | 30                   | 46.1                                      |
|                                      | 60                   | 53.3                                      |
| Triethanolamine.....                 | 30                   | 20.6                                      |
|                                      | 60                   | 21.5                                      |
| Triethylamine.....                   | 30                   | 15.1                                      |
|                                      | 60                   | 16.2                                      |
| Triallylamine.....                   | 30                   | 11.6                                      |
|                                      | 60                   | 11.7                                      |

From the results of the measurement it will be seen that chemical treatments employing monoethylamine, diethylamine both amines of monoethylamine and diethylamine and monoethanolamine resulted in coatings of considerable thicknesses.

#### (2) Alkali resistance test

Aluminum specimens treated as described above were immersed in a 0.1 N solution of caustic soda heated to 35°C. and the difference between the weight after lapse of a given period of time and the weight before the test was measured to observe the alkali resistance of the specimens. The test of aluminum specimens chemically

treated by using both amines of monoethylamine and diethylamine was omitted.

| Additives           | Treating time (min.) | Weight of coating (mg./dm. <sup>2</sup> ) | 5          |
|---------------------|----------------------|-------------------------------------------|------------|
| Present invention:  |                      |                                           |            |
| Monoethylamine      | 30                   | 4.2                                       | 106.9      |
|                     | 60                   | 2.4                                       | 51.5       |
| Diethylamine        | 30                   | 5.6                                       | 89.0       |
|                     | 60                   | 5.6                                       | 79.4 10    |
| Reference examples: |                      |                                           |            |
| Monoethanolamine    | 30                   | 6.7                                       | 105.0      |
|                     | 60                   | 3.6                                       | 62.7       |
| Triethanolamine     | 30                   | 12.7                                      | 207.3      |
|                     | 60                   | 7.8                                       | 111.7      |
| Triethylamine       | 30                   | 24.0                                      | 452.2      |
|                     | 60                   | 17.6                                      | 348.1      |
| Triallylamine       | 30                   | 41.7                                      | 1,573.9 15 |
|                     | 60                   | 29.5                                      | 1,137.1    |

From the test results it will be noted that high resistance to alkali was effected by chemical treatments which employed monoethylamine, diethylamine and mono-ethanolamine. 20

### (3) Acid resistance test

The specimens were immersed in a 0.5 N solution of hydrochloric acid heated to 35° C. and the difference between the weight after lapse of a given period of time and the weight before the test was measured to observe the acid resistance of the specimens. The test of aluminum specimens chemically treated by using both amines of monoethylamine and diethylamine was omitted. 25 30

| Additives           | Treating time (min.) | Weight reduction in 3 hrs. (mg./dm. <sup>2</sup> ) | Weight reduction in 10 hrs. (mg./dm. <sup>2</sup> ) | 35 |
|---------------------|----------------------|----------------------------------------------------|-----------------------------------------------------|----|
| Present invention:  |                      |                                                    |                                                     |    |
| Monoethylamine      | 30                   | 2.0                                                | 18.4                                                |    |
|                     | 60                   | 1.9                                                | 16.7                                                |    |
| Diethylamine        | 30                   | 5.1                                                | 595.9                                               |    |
|                     | 60                   | 4.7                                                | 528.5 40                                            |    |
| Reference examples: |                      |                                                    |                                                     |    |
| Monoethanolamine    | 30                   | 8.3                                                | 1,629.6                                             |    |
|                     | 60                   | 12.7                                               | 2,221.1                                             |    |
| Triethanolamine     | 30                   | 6.9                                                | 904.0                                               |    |
|                     | 60                   | 2.8                                                | 811.7                                               |    |
| Triethylamine       | 30                   | 7.3                                                | 796.7                                               |    |
|                     | 60                   | 7.3                                                | 831.9                                               |    |
| Triallylamine       | 30                   | 13.5                                               | 2,180.1                                             |    |
|                     | 60                   | 11.2                                               | 2,123.7 45                                          |    |

The test results show that superior resistance to acid was obtained by chemical treatments employing monoethylamine and diethylamine. 50

As apparent from the results of the foregoing tests the specimens chemically treated in accordance with the present invention have thick coatings which are excellent in resistance to alkali and to acid.

### EXAMPLE 2

Pretreatment and aftertreatment were conducted under the same conditions as in Example 1. In carrying out treatments in accordance with the present invention, monoethylamine, diethylamine and both amines of monoethylamine and diethylamine were added in different amounts of 0.5, 3, 12, 24, 30 cc./liter. The weight of coating and resistance to alkali and to acid were measured with respect to the specimens thus treated. The results are given below. 60

As reference examples, treatments were conducted using triethanolamine which is commonly used. The results are also shown.

#### (1) Measurement of weight of coating

After the formation of chemical coating, the specimens were immersed in a boiling stripping solution of phosphoric acid-chromic acid. Based upon the difference of weight produced by the immersion, the weight of coating was measured to observe the state of the coating formed. 70 75

| Additives                       | Amount added (cc./liter) | Treating time (min.) | Weight of coating (mg./dm. <sup>2</sup> ) |
|---------------------------------|--------------------------|----------------------|-------------------------------------------|
| Present invention:              |                          |                      |                                           |
| Monoethylamine                  | 0.5                      | 5                    | 30.2                                      |
|                                 |                          | 10                   | 33.8                                      |
|                                 |                          | 15                   | 37.5                                      |
|                                 |                          | 30                   | 38.4                                      |
|                                 |                          | 60                   | 39.5                                      |
|                                 |                          | 5                    | 39.9                                      |
|                                 |                          | 10                   | 43.3                                      |
|                                 | 3                        | 15                   | 48.2                                      |
|                                 |                          | 30                   | 57.0                                      |
|                                 |                          | 60                   | 58.4                                      |
|                                 |                          | 5                    | 54.7                                      |
|                                 |                          | 10                   | 68.6                                      |
|                                 |                          | 15                   | 83.3                                      |
|                                 |                          | 30                   | 104.2                                     |
|                                 |                          | 60                   | 124.0                                     |
|                                 |                          | 5                    | 68.5                                      |
|                                 |                          | 10                   | 84.2                                      |
|                                 |                          | 15                   | 101.6                                     |
|                                 |                          | 30                   | 128.2                                     |
|                                 |                          | 60                   | 155.0                                     |
|                                 |                          | 5                    | 79.4                                      |
|                                 |                          | 10                   | 96.8                                      |
|                                 | 30                       | 15                   | 116.8                                     |
|                                 |                          | 30                   | 147.7                                     |
|                                 |                          | 60                   | 178.2                                     |
|                                 |                          | 5                    | 21.0                                      |
|                                 |                          | 10                   | 21.5                                      |
|                                 | 0.5                      | 15                   | 22.9                                      |
|                                 |                          | 30                   | 23.2                                      |
|                                 |                          | 60                   | 24.3                                      |
|                                 |                          | 5                    | 29.5                                      |
|                                 |                          | 10                   | 31.0                                      |
|                                 | 3                        | 15                   | 32.4                                      |
|                                 |                          | 30                   | 33.4                                      |
|                                 |                          | 60                   | 35.2                                      |
|                                 |                          | 5                    | 44.1                                      |
|                                 |                          | 10                   | 51.0                                      |
|                                 |                          | 15                   | 57.1                                      |
|                                 |                          | 30                   | 58.0                                      |
|                                 |                          | 60                   | 61.0                                      |
|                                 |                          | 5                    | 54.2                                      |
|                                 |                          | 10                   | 63.5                                      |
|                                 |                          | 15                   | 70.0                                      |
|                                 |                          | 30                   | 82.0                                      |
|                                 |                          | 60                   | 85.7                                      |
|                                 |                          | 5                    | 67.3                                      |
|                                 |                          | 10                   | 75.5                                      |
|                                 | 30                       | 15                   | 85.7                                      |
|                                 |                          | 30                   | 90.6                                      |
|                                 |                          | 60                   | 97.1                                      |
|                                 |                          | 5                    | 28.0                                      |
|                                 |                          | 10                   | 31.7                                      |
|                                 | 0.5                      | 15                   | 36.1                                      |
|                                 |                          | 30                   | 36.2                                      |
|                                 |                          | 60                   | 36.3                                      |
|                                 |                          | 5                    | 39.1                                      |
|                                 |                          | 10                   | 40.6                                      |
|                                 | 3                        | 15                   | 44.7                                      |
|                                 |                          | 30                   | 50.4                                      |
|                                 |                          | 60                   | 52.0                                      |
|                                 |                          | 5                    | 51.1                                      |
|                                 |                          | 10                   | 54.3                                      |
|                                 |                          | 15                   | 65.0                                      |
|                                 |                          | 30                   | 83.7                                      |
|                                 |                          | 60                   | 103.0                                     |
|                                 |                          | 5                    | 52.7                                      |
|                                 |                          | 10                   | 70.3                                      |
|                                 |                          | 15                   | 88.0                                      |
|                                 |                          | 30                   | 114.4                                     |
|                                 |                          | 60                   | 140.0                                     |
|                                 |                          | 5                    | 66.5                                      |
|                                 |                          | 10                   | 83.8                                      |
|                                 | 30                       | 15                   | 91.9                                      |
|                                 |                          | 30                   | 132.4                                     |
|                                 |                          | 60                   | 160.2                                     |
| Reference example:              |                          |                      |                                           |
| Monoethylamine and diethylamine | 12                       | 5                    | 9.2                                       |
|                                 |                          | 10                   | 10.4                                      |
|                                 | 0.5                      | 15                   | 12.8                                      |
|                                 |                          | 30                   | 13.9                                      |
|                                 |                          | 60                   | 14.8                                      |
|                                 |                          | 5                    | 15.9                                      |
|                                 |                          | 10                   | 17.1                                      |
|                                 | 3                        | 15                   | 19.8                                      |
|                                 |                          | 30                   | 20.6                                      |
|                                 |                          | 60                   | 21.5                                      |
|                                 |                          | 5                    | 28.5                                      |
|                                 |                          | 10                   | 30.3                                      |
|                                 | 12                       | 15                   | 32.5                                      |
|                                 |                          | 30                   | 33.7                                      |
|                                 |                          | 60                   | 36.8                                      |
|                                 |                          | 5                    | 32.2                                      |
|                                 |                          | 10                   | 35.7                                      |
|                                 | 24                       | 15                   | 36.5                                      |
|                                 |                          | 30                   | 38.5                                      |
|                                 |                          | 60                   | 38.8                                      |
|                                 |                          | 5                    | 34.9                                      |
|                                 |                          | 10                   | 35.9                                      |
|                                 | 30                       | 15                   | 36.9                                      |
|                                 |                          | 30                   | 38.6                                      |
|                                 |                          | 60                   | 39.1                                      |

From the results of the measurement it will be seen that the chemical treatments of the present invention employing monoethylamine, diethylamine and both amines

of monoethylamine and diethylamine resulted in coatings which were thicker than those obtained by using triethanolamine.

(2) Alkali resistance test

Specimens were immersed in a 0.5 N solution of cau-

tic soda heated to 35° C. and the difference between the weight after lapse of a given period of time and the weight before the test was measured to observe the alkali resistance of the specimens.

| Additives                       | Amount added<br>(cc./liter) | Treating time<br>(min.) | Weight reduction (mg./dm. <sup>2</sup> ) in— |         |         |
|---------------------------------|-----------------------------|-------------------------|----------------------------------------------|---------|---------|
|                                 |                             |                         | 1 hour                                       | 2 hours | 3 hours |
| Present invention:              |                             |                         |                                              |         |         |
| Monoethylamine                  |                             |                         |                                              |         |         |
|                                 | 0.5                         | 5                       | 321.3                                        |         |         |
|                                 |                             | 10                      | 198.2                                        |         |         |
|                                 |                             | 15                      | 53.8                                         |         |         |
|                                 |                             | 30                      | 4.2                                          | 44.8    |         |
|                                 |                             | 60                      | 4.1                                          | 40.7    |         |
|                                 |                             | 5                       | 99.5                                         |         |         |
|                                 |                             | 10                      | 64.0                                         |         |         |
|                                 | 3                           | 15                      | 13.1                                         | 277.5   |         |
|                                 |                             | 30                      | 2.6                                          | 25.7    | 92.3    |
|                                 |                             | 60                      | 2.5                                          | 13.0    | 39.8    |
|                                 |                             | 5                       | 90.7                                         |         |         |
|                                 |                             | 10                      | 50.1                                         |         |         |
|                                 | 12                          | 15                      | 3.6                                          | 93.2    |         |
|                                 |                             | 30                      | 2.4                                          | 11.4    | 69.2    |
|                                 |                             | 60                      | 2.1                                          | 9.8     | 32.3    |
|                                 |                             | 5                       | 80.6                                         |         |         |
|                                 |                             | 10                      | 29.6                                         | 192.8   |         |
|                                 | 24                          | 15                      | 1.6                                          | 29.8    |         |
|                                 |                             | 30                      | 1.5                                          | 11.1    | 67.8    |
|                                 |                             | 60                      | 1.3                                          | 7.7     | 29.7    |
|                                 |                             | 5                       | 45.9                                         | 740.5   |         |
|                                 | 30                          | 10                      | 28.3                                         | 160.4   |         |
|                                 |                             | 15                      | 1.6                                          | 21.2    | 1,125.0 |
|                                 |                             | 30                      | 1.4                                          | 10.2    | 50.8    |
|                                 |                             | 60                      | 1.2                                          | 6.1     | 19.8    |
| Diethylamine                    |                             |                         |                                              |         |         |
|                                 | 0.5                         | 5                       | 699.2                                        |         |         |
|                                 |                             | 10                      | 116.2                                        |         |         |
|                                 |                             | 15                      | 59.3                                         |         |         |
|                                 |                             | 30                      | 24.3                                         |         |         |
|                                 |                             | 60                      | 23.5                                         | 696.5   |         |
|                                 |                             | 5                       | 73.3                                         |         |         |
|                                 |                             | 10                      | 39.8                                         |         |         |
|                                 | 3                           | 15                      | 11.1                                         | 103.0   |         |
|                                 |                             | 30                      | 7.5                                          | 40.1    |         |
|                                 |                             | 60                      | 5.2                                          | 38.8    |         |
|                                 |                             | 5                       | 47.5                                         |         |         |
|                                 |                             | 10                      | 14.5                                         | 88.2    |         |
|                                 | 12                          | 15                      | 7.2                                          | 57.2    |         |
|                                 |                             | 30                      | 3.8                                          | 32.5    | 110.2   |
|                                 |                             | 60                      | 3.5                                          | 23.3    | 90.7    |
|                                 |                             | 5                       | 44.1                                         |         |         |
|                                 |                             | 10                      | 7.0                                          | 50.2    |         |
|                                 | 24                          | 15                      | 4.4                                          | 42.6    | 729.8   |
|                                 |                             | 30                      | 3.3                                          | 29.7    | 98.6    |
|                                 |                             | 60                      | 2.7                                          | 28.2    | 79.2    |
|                                 |                             | 5                       | 21.3                                         | 89.7    |         |
|                                 |                             | 10                      | 6.2                                          | 42.9    | 976.0   |
|                                 | 30                          | 15                      | 3.9                                          | 40.2    | 512.7   |
|                                 |                             | 30                      | 2.7                                          | 27.6    | 82.6    |
|                                 |                             | 60                      | 2.5                                          | 24.1    | 60.8    |
| Monoethylamine and diethylamine |                             |                         |                                              |         |         |
|                                 | 0.5                         | 5                       | 2,282.5                                      |         |         |
|                                 |                             | 10                      | 234.1                                        |         |         |
|                                 |                             | 15                      | 47.1                                         |         |         |
|                                 |                             | 30                      | 13.5                                         | 144.0   |         |
|                                 |                             | 60                      | 5.7                                          | 9.1     | 30.6    |
|                                 |                             | 5                       | 576.2                                        |         |         |
|                                 |                             | 10                      | 59.1                                         |         |         |
|                                 | 3                           | 15                      | 11.9                                         | 155.7   |         |
|                                 |                             | 30                      | 8.4                                          | 73.1    |         |
|                                 |                             | 60                      | 4.6                                          | 7.9     | 24.2    |
|                                 |                             | 5                       | 180.9                                        |         |         |
|                                 |                             | 10                      | 25.8                                         | 417.8   |         |
|                                 | 12                          | 15                      | 05.8                                         | 96.1    | 408.8   |
|                                 |                             | 30                      | 4.8                                          | 43.4    | 91.3    |
|                                 |                             | 60                      | 4.0                                          | 7.3     | 23.6    |
|                                 |                             | 5                       | 125.8                                        |         |         |
|                                 |                             | 10                      | 12.9                                         | 277.2   |         |
|                                 | 24                          | 15                      | 5.6                                          | 55.9    | 283.6   |
|                                 |                             | 30                      | 4.3                                          | 40.9    | 79.8    |
|                                 |                             | 60                      | 4.0                                          | 6.9     | 22.5    |
|                                 |                             | 5                       | 115.4                                        |         |         |
|                                 |                             | 10                      | 11.8                                         | 220.6   |         |
|                                 | 30                          | 15                      | 5.4                                          | 51.6    | 187.6   |
|                                 |                             | 30                      | 4.1                                          | 32.6    | 45.6    |
|                                 |                             | 60                      | 3.2                                          | 6.1     | 21.8    |

TABLE—Continued

| Additives          | Amount added<br>(cc./liter) | Treating time<br>(min.) | Weight reduction (mg./dm. <sup>2</sup> ) in— |         |         |
|--------------------|-----------------------------|-------------------------|----------------------------------------------|---------|---------|
|                    |                             |                         | 1 hour                                       | 2 hours | 3 hours |
| Reference example: |                             |                         |                                              |         |         |
| Triethanolamine    | 0.5                         | 5                       |                                              |         |         |
|                    |                             | 10                      | 3,871.2                                      |         |         |
|                    |                             | 15                      | 779.0                                        |         |         |
|                    |                             | 30                      | 374.5                                        |         |         |
|                    |                             | 60                      | 299.6                                        |         |         |
|                    | 3                           | 5                       |                                              |         |         |
|                    |                             | 10                      | 2,275.8                                      |         |         |
|                    |                             | 15                      | 457.9                                        |         |         |
|                    |                             | 30                      | 216.5                                        |         |         |
|                    |                             | 60                      | 166.5                                        |         |         |
|                    | 12                          | 5                       | 1,344.2                                      |         |         |
|                    |                             | 10                      | 185.4                                        |         |         |
|                    |                             | 15                      | 37.3                                         | 828.8   |         |
|                    |                             | 30                      | 17.0                                         | 516.7   |         |
|                    |                             | 60                      | 8.4                                          | 215.1   |         |
|                    | 24                          | 5                       | 424.0                                        |         |         |
|                    |                             | 10                      | 58.6                                         |         |         |
|                    |                             | 15                      | 11.8                                         | 192.8   |         |
|                    |                             | 30                      | 6.5                                          | 103.0   |         |
|                    |                             | 60                      | 5.5                                          | 51.5    |         |
|                    | 30                          | 5                       | 342.4                                        |         |         |
|                    |                             | 10                      | 52.4                                         |         |         |
|                    |                             | 15                      | 10.4                                         | 120.9   |         |
|                    |                             | 30                      | 5.1                                          | 97.2    |         |
|                    |                             | 60                      | 5.3                                          | 50.9    |         |

It will be apparent from the test results that the chemical treatments of the present invention employing monoethylamine, diethylamine and both amines of monoethylamine and diethylamine produced coatings which were higher in alkali resistance than those obtained by using triethanolamine.

### (3) Acid resistance test

30 The specimens were immersed in a 0.5 N solution of hydrochloric acid heated to 35° C. and the difference between the weight after lapse of a given period of time and the weight before the test was measured to observe the acid resistance of the specimens.

| Additives          | Amount added<br>(cc./liter) | Treating time<br>(min.) | Weight reduction (mg./dm. <sup>2</sup> ) in— |         |          |
|--------------------|-----------------------------|-------------------------|----------------------------------------------|---------|----------|
|                    |                             |                         | 4 hour                                       | 8 hours | 14 hours |
| Present invention: |                             |                         |                                              |         |          |
| Monoethylamine     | 0.5                         | 5                       | 13.5                                         | 332.7   |          |
|                    |                             | 10                      | 12.4                                         | 287.6   |          |
|                    |                             | 15                      | 10.9                                         | 270.9   |          |
|                    |                             | 30                      | 7.0                                          | 220.4   |          |
|                    |                             | 60                      | 6.9                                          | 158.3   |          |
|                    | 3                           | 5                       | 7.1                                          | 81.8    |          |
|                    |                             | 10                      | 6.8                                          | 70.4    |          |
|                    |                             | 15                      | 4.2                                          | 27.9    | 972.5    |
|                    |                             | 30                      | 2.7                                          | 11.7    | 320.7    |
|                    |                             | 60                      | 2.6                                          | 9.8     | 89.6     |
|                    | 12                          | 5                       | 4.9                                          | 22.7    | 72.0     |
|                    |                             | 10                      | 4.2                                          | 14.3    | 49.2     |
|                    |                             | 15                      | 2.3                                          | 8.1     | 26.3     |
|                    |                             | 30                      | 2.1                                          | 6.4     | 23.4     |
|                    |                             | 60                      | 2.0                                          | 6.3     | 21.5     |
|                    | 24                          | 5                       | 3.7                                          | 12.9    | 36.3     |
|                    |                             | 10                      | 3.2                                          | 10.8    | 29.8     |
|                    |                             | 15                      | 2.2                                          | 7.9     | 26.1     |
|                    |                             | 30                      | 1.8                                          | 6.1     | 23.2     |
|                    |                             | 60                      | 1.7                                          | 6.0     | 21.0     |
|                    | 30                          | 5                       | 4.2                                          | 14.9    | 38.8     |
|                    |                             | 10                      | 3.9                                          | 13.1    | 31.6     |
|                    |                             | 15                      | 2.8                                          | 9.7     | 25.9     |
|                    |                             | 30                      | 2.6                                          | 8.2     | 23.3     |
|                    |                             | 60                      | 2.1                                          | 7.8     | 23.1     |
|                    |                             | 5                       | 16.9                                         | 652.3   |          |
|                    | 0.5                         | 10                      | 14.2                                         | 548.1   |          |
|                    |                             | 15                      | 12.8                                         | 436.2   |          |
|                    |                             | 30                      | 11.8                                         | 425.0   |          |
|                    |                             | 60                      | 10.9                                         | 351.8   |          |
|                    | 3                           | 5                       | 11.1                                         | 325.3   |          |
|                    |                             | 10                      | 10.6                                         | 322.5   |          |
|                    |                             | 15                      | 9.8                                          | 129.7   |          |
|                    |                             | 30                      | 7.6                                          | 111.8   |          |
|                    |                             | 60                      | 6.2                                          | 98.8    |          |
|                    | 12                          | 5                       | 3.8                                          | 16.5    | 698.8    |
|                    |                             | 10                      | 3.7                                          | 9.6     | 232.3    |
|                    |                             | 15                      | 2.4                                          | 6.1     | 30.8     |
|                    |                             | 30                      | 2.0                                          | 5.9     | 21.7     |
|                    | 24                          | 5                       | 1.5                                          | 9.7     | 28.4     |
|                    |                             | 10                      | 1.5                                          | 9.3     | 22.9     |
|                    |                             | 15                      | 1.2                                          | 5.9     | 18.6     |
|                    |                             | 30                      | 0.7                                          | 5.1     | 14.9     |
|                    |                             | 60                      | 0.7                                          | 5.0     | 12.7     |
|                    | 30                          | 5                       | 4.3                                          | 14.4    | 33.3     |
|                    |                             | 10                      | 4.1                                          | 14.2    | 32.9     |
|                    |                             | 15                      | 3.2                                          | 7.5     | 17.4     |
|                    |                             | 30                      | 3.2                                          | 6.6     | 15.5     |
|                    |                             | 60                      | 3.0                                          | 6.2     | 14.4     |

TABLE—Continued

| Additives                       | Amount added<br>(cc./liter) | Treating time<br>(min.) | Weight reduction (mg./dm. <sup>2</sup> ) in— |         |          |
|---------------------------------|-----------------------------|-------------------------|----------------------------------------------|---------|----------|
|                                 |                             |                         | 4 hour                                       | 8 hours | 14 hours |
| Monoethylamine and diethylamine | 0.5                         | 5                       | 9.9                                          | 323.6   | -----    |
|                                 |                             | 10                      | 8.3                                          | 297.3   | -----    |
|                                 |                             | 15                      | 6.8                                          | 244.6   | -----    |
|                                 |                             | 30                      | 6.3                                          | 237.1   | -----    |
|                                 |                             | 60                      | 5.9                                          | 231.2   | -----    |
|                                 |                             | 5                       | 5.7                                          | 100.2   | -----    |
|                                 | 3                           | 10                      | 5.4                                          | 92.9    | -----    |
|                                 |                             | 15                      | 4.4                                          | 81.9    | 869.3    |
|                                 |                             | 30                      | 4.3                                          | 79.1    | 720.1    |
|                                 |                             | 60                      | 4.1                                          | 60.8    | 431.7    |
|                                 |                             | 5                       | 4.6                                          | 10.8    | 57.6     |
|                                 |                             | 10                      | 4.1                                          | 9.2     | 47.0     |
| Reference example:              | 12                          | 15                      | 3.9                                          | 8.1     | 28.8     |
|                                 |                             | 30                      | 3.7                                          | 7.4     | 16.3     |
|                                 |                             | 60                      | 3.2                                          | 7.2     | 15.0     |
|                                 |                             | 5                       | 4.2                                          | 9.1     | 45.7     |
|                                 |                             | 10                      | 4.0                                          | 8.5     | 40.2     |
|                                 |                             | 24                      | 3.8                                          | 8.0     | 24.9     |
|                                 | 24                          | 30                      | 3.5                                          | 7.1     | 15.7     |
|                                 |                             | 60                      | 3.0                                          | 6.7     | 13.3     |
|                                 |                             | 5                       | 7.4                                          | 10.7    | 72.6     |
|                                 |                             | 10                      | 7.2                                          | 9.8     | 39.7     |
|                                 |                             | 30                      | 7.2                                          | 9.1     | 30.3     |
|                                 |                             | 60                      | 6.8                                          | 8.2     | 22.6     |
|                                 |                             | 60                      | 6.8                                          | 7.7     | 20.4     |
| Triethanolamine                 | 0.5                         | 5                       | 364.6                                        | -----   | -----    |
|                                 |                             | 10                      | 277.5                                        | -----   | -----    |
|                                 |                             | 15                      | 145.6                                        | -----   | -----    |
|                                 |                             | 30                      | 75.8                                         | -----   | -----    |
|                                 |                             | 60                      | 30.5                                         | -----   | -----    |
|                                 |                             | 5                       | 44.6                                         | 604.9   | -----    |
|                                 | 3                           | 10                      | 38.7                                         | 430.3   | -----    |
|                                 |                             | 15                      | 13.8                                         | 673.9   | -----    |
|                                 |                             | 30                      | 7.8                                          | 437.2   | -----    |
|                                 |                             | 60                      | 3.9                                          | 412.6   | -----    |
|                                 |                             | 5                       | 4.6                                          | 381.7   | -----    |
|                                 |                             | 10                      | 4.4                                          | 354.5   | -----    |
|                                 | 12                          | 15                      | 4.7                                          | 222.0   | -----    |
|                                 |                             | 30                      | 10.6                                         | 442.0   | -----    |
|                                 |                             | 60                      | 16.4                                         | 533.3   | -----    |
|                                 |                             | 5                       | 5.3                                          | 333.6   | -----    |
|                                 |                             | 10                      | 5.6                                          | 327.8   | -----    |
|                                 |                             | 24                      | 15.9                                         | 422.7   | -----    |
|                                 | 24                          | 30                      | 18.5                                         | 470.4   | -----    |
|                                 |                             | 60                      | 26.0                                         | 613.9   | -----    |
|                                 |                             | 5                       | 8.7                                          | 341.3   | -----    |
|                                 |                             | 10                      | 10.4                                         | 420.0   | -----    |
|                                 |                             | 30                      | 20.0                                         | 500.7   | -----    |
|                                 |                             | 60                      | 22.7                                         | 537.1   | -----    |
|                                 |                             | 60                      | 30.3                                         | 687.6   | -----    |

It will be noted from the test results that the chemical coatings formed in accordance with the present invention have higher resistance to acid than those formed by using triethanolamine.

As apparent from the results of the respective tests stated above, the specimens subjected to the chemical treatment of the present invention are more excellent than those obtained by using triethanolamine with respect to the state of the coating formed and resistance to alkali and to acid.

While in the foregoing specification, a detailed description of a specific embodiment of our invention was set forth for the purpose of illustration, it is to be understood that many of the details herein given may be varied considerably by those skilled in the art without departing from the spirit and scope of our invention.

We claim:

1. A method for forming a boehmite-containing chemical coating on a metal selected from the class of aluminum and aluminum alloy comprising the steps of im-

mersing the metal in a heated aqueous solution consisting of water and at least one member selected from the class of monoethylamine and diethylamine for about 5 to about 60 minutes, said solution having a concentration of from 0.5 to 30 cc. of said members per liter of water, and subjecting the metal to pressurized steam after the metal is removed from the aqueous solution.

#### References Cited

##### UNITED STATES PATENTS

50 3,380,860 4/1963 Lipinski ----- 148—6.27  
3,544,391 12/1970 Scott ----- 148—6.27

##### FOREIGN PATENTS

719,680 10/1965 Canada ----- 148—6.27

55 RALPH S. KENDALL, Primary Examiner

U.S. CL. X.R.

148—6.3